

## UNITED STATES PATENT OFFICE

1,934,789

PRODUCTION OF FAST COLOR RESERVES  
UNDER GROUND DYEINGS

Philippe Brandt, Mulhouse, Haut-Rhin, France,  
and Emil Gubler and Ernst Tschan, Basel,  
Switzerland, assignors to firm Durand &  
Huguenin S. A., Basel, Switzerland

No Drawing. Application October 10, 1931,  
Serial No. 568,202, and in Germany October 10,  
1930

## 5 Claims. (CL. 8—5)

In the U. S. patent application Ser. No. 554,945, filed August 3, 1931, a process for producing fast color reserves under ground dyeings is described in which a steaming operation for developing the dyestuff is avoided. According to the said process it is possible to produce such color reserves under ground dyeings with the aid of ester-salts of leuco-vat-dyestuffs (see U. S. Patent No. 1,448,251) by printing on a material impregnated with an arylide of 2:3-hydroxy-naphthoic acid a reserve color containing an ester-salt of a leuco-vat-dyestuff and, besides the usual additions, an acid reacting salt, drying and afterwards padding the material in a solution of a diazotized 4-amino-15 diphenylamine compound in order to produce the ground dyeing. Finally the ester-salt is developed by passing the material through an acid bath containing a mild oxidizing agent.

Surprisingly it has now been found, that such color reserves with the aid of ester salts of leuco vat dyestuffs can be produced in a still simpler way, without any steaming operation and without an acid developing bath, by means of a drying operation only. According to the invention aluminium chloride is printed on the naphtholated material simultaneously with the ester salt and an acid reacting salt. The material is then subjected to a drying operation, whereby the color reserves are developed. Finally the ground dyeing is produced by padding the material in a solution of a diazo compound.

As a number of ester-salts require some time for their development, as the case may be, the goods are left lying for a certain time after 35 drying.

The developing time can be shortened, that is to say, the developing power of the aluminium chloride may be increased by the presence of an oxidizing catalyst, such as for instance ammonium vanadate, osmium tetroxide, potassium ferricyanide, a copper-salt, brought on to the fibre previously or simultaneously with the naphthol or in any other step of the process. The above mentioned catalysts may also be used in combination with each other.

In the German Patent No. 525,302 the use of aluminium chloride as developer for leuco-vat-dyestuffs has already been recommended, but according to the process described therein the development is initiated by steaming. In the present new process no steaming operation is required.

The invention does not only represent a simpli-

fication but also a considerable improvement over the prior art inasmuch as the use of aluminium chloride does not act as developing agent only, but it helps to improve the reserve-efficiency of the acid reacting salt. It is therefore possible to economize on this product.

Furthermore in the earlier process, wherein the development of the ester-salt-reserves followed the development of the ground dyeing, the latter was more or less affected by the oxidizing agents, so that it was necessary to choose a mild one. But as certain ester-salts require more powerful oxidizing agents for their development, it is clear, that hitherto the choice of these dyestuffs for color reserve purposes has been limited.

This disadvantage has been overcome, since, contrarily to the prior process, it has been found, that the developer, in this case aluminium chloride, acts only locally and not on the whole material and is capable of developing practically the whole of the ester-salts of leuco-vat-dyestuffs. As the color reserves are developed before the ground dyeing, there is no more danger for the latter to be damaged.

Besides ester-salt-reserves other color-reserves, for instance when printing a preparation of a diazotized para-nitraniline compound on the material, red reserves may be obtained. The variety of the effects which can be produced may still be increased, when using other suitable dyestuffs.

The new process is illustrated by the following examples.

## Example 1

On the material padded with the anilide of 2:3-hydroxy-naphthoic acid in the usual way, there is printed, after drying, a color of the following composition:

|                                                                     | Parts |
|---------------------------------------------------------------------|-------|
| Sodium salt of the disulphuric acid ester of leuco-tetra-bromindigo | 2     |
| Thio-methylene-glycol                                               | 6 95  |
| Water                                                               | 30    |
| Neutral-starch and gum tragacanth thickening                        | 50    |
| Solution of aluminium sulphate (1:1)                                | 4     |
| Solution of aluminium chloride (25° Bé.)                            | 8 100 |
|                                                                     | 100   |

The material is dried at 60° to 70° C. in a drying chamber or on the drum, left lying for 24 hours, whereby the light blue reserve effect, orig-

- inating in the ester of leuco-tetra-bromindigo is developed. After drying, the material is padded in a solution containing the diazo compound of 4-amino-4'-methoxy-diphenylamine. 5 Then an air passage for 30 to 60 seconds is applied, whereby the development of the ground dyeing takes place. To destroy any excess of the diazo compound, the material is treated for 5 minutes in a bath of 60° C. containing 5 ccm. 10 of muriatic acid per litre of water, thoroughly rinsed and dried. A fast light blue on a navy ground is obtained.

*Example 2*

- 15 On the material padded with the anilide of 2:3-hydroxy-naphthoic acid in the usual way, there is printed, after drying, a color of the following composition:

|                                                                            | Parts |
|----------------------------------------------------------------------------|-------|
| 20 Sodium salt of the disulphuric acid ester of leuco-dibenzopyrenequinone | 4     |
| Thio-diethylene-glycol                                                     | 6     |
| Water                                                                      | 27, 8 |
| Neutral-starch and gum tragacanth thick-<br>ening                          | 50    |
| 25 Solution of aluminium sulphate (1:1)                                    | 6     |
| Solution of aluminium chloride (25° Bé.)                                   | 6     |
| Oxalic acid                                                                | 0, 2  |
|                                                                            | 100   |
| 30                                                                         |       |

The material is dried at a temperature of 60 to 70° C. in a drying chamber or on the drum. During this drying operation the ester-salt is developed completely. The ground dyeing is produced and the goods are finally treated as in Example 1. Thus yellow reserves on a navy ground are obtained.

*Example 3*

- 40 The following printing color is prepared:

|                                                                            | Parts |
|----------------------------------------------------------------------------|-------|
| Sodium salt of the disulphuric acid ester of leuco-dimethoxydibenzanthrone | 8     |
| Thio-diethylene-glycol                                                     | 6     |
| 45 Water                                                                   | 24    |
| Neutral starch and gum tragacanth thick-<br>ening                          | 50    |
| Solution of aluminium sulphate (1:1)                                       | 4     |
| Solution of aluminium chloride (25° Bé.)                                   | 8     |
| 50                                                                         |       |

This color is printed on cotton material, previously padded with the anilide of 2:3-hydroxy-naphthoic acid. The material is afterwards dried at 60 to 70° C. in a drying chamber or on the drum, whereby the green color reserve is developed. The ground dyeing is produced by means of a solution of diazo-4-amino-4'-methoxy-diphenylamine as stated in Example 1. Thus a fast green 60 on a navy ground results.

*Example 4*

The material is first padded in a bath of the following composition:

|                                                                             | Parts |                              |
|-----------------------------------------------------------------------------|-------|------------------------------|
| Anilide of the 2:3-hydroxy-naph-<br>thoic acid                              | 17, 5 | Dissolved<br>in hot<br>water |
| Caustic soda lye (34° Bé.)                                                  | 20    |                              |
| Ricino-sulphonic acid                                                       | 16    |                              |
| 70 Sodium salt of the 1-isopropyl-<br>naphthalene-4-sulphonic acid<br>(10%) | 15    |                              |
| Ammonium vanadate (1%)                                                      | 100   |                              |

75 the whole diluted with water to 1 litre.

After drying there is printed on a color composed as follows:

|                                                                 | Parts |
|-----------------------------------------------------------------|-------|
| Sodium salt of the disulphuric acid ester of 2:1-naphthioindigo | 2     |
| Thio-diethylene-glycol                                          | 5     |
| Sodium salt of benzyl-aniline sulphonic acid                    | 5     |
| Diethyl ether of diethylene-glycol                              | 5     |
| Warm water                                                      | 17    |
| Neutral-starch and gum tragacanth thick-<br>ening               | 85    |
| Solution of aluminium sulphate (1:1)                            | 4     |
| Solution of aluminium chloride (25° Bé.)                        | 12    |
|                                                                 | 100   |
|                                                                 | 90    |

The material is dried at 60 to 70° C. in a drying chamber or on the drum and left lying for 24 hours, whereby the ester salt is developed. Afterwards the ground dyeing is produced and the goods are finally treated as stated in Example 1. 95 A fast brown reserve on navy ground is obtained.

In a similar manner color reserves on navy ground may be obtained by printing on the following ester-salts of leuco-vat-dyestuffs:

Sodium salt of the disulphuric acid ester of isatin anilide and 1-methyl-7:8-oxybenzocarbazol:—giving grey to black effects.

Sodium salt of the disulphuric acid ester of leuco-6:5':7-trichlorindigo:—giving violet effects.

In the aforesaid examples instead of aluminium sulphate another acid reacting salt, for instance zinc sulphate, may be used with a similar effect.

What we claim is:

1. A process for producing fast color reserves 110 under ground dyeings by means of ester salts of leuco vat dyestuffs without steaming, consisting in taking a fabric impregnated with an arylide of 2:3-hydroxy-naphthoic acid, printing thereon a reserve color containing an ester salt of 115 a leuco vat dyestuff, aluminium chloride as oxidizing agent and an acid reacting salt, thereupon drying the material, whereby the color reserve is developed, and afterwards padding the same in a solution of a diazotized 4-amino-di- 120 phenylamine compound in order to produce the ground dyeing.

2. A process for producing fast color reserves 125 under ground dyeings by means of ester salts of leuco vat dyestuffs without steaming, consisting in taking a fabric impregnated with an arylide of 2:3-hydroxy-naphthoic acid, printing thereon a reserve color containing an ester salt of a leuco vat dyestuff, aluminium chloride as oxidizing agent and aluminium sulphate as acid reacting salt, thereupon drying the material, whereby the color reserve is developed, and afterwards padding the same in a solution of a diazotized 4-amino-di- 130 phenylamine compound in order to produce the ground dyeing.

3. A process for producing fast color reserves 135 underground dyeings by means of ester salts of leuco vat dyestuffs without steaming, consisting in taking a fabric impregnated with an arylide of 2:3-hydroxy-naphthoic acid, printing thereon a reserve color containing an ester salt of a leuco vat dyestuff, aluminium chloride as oxidizing agent, a catalyst and an acid reacting salt, thereupon drying the material, whereby the color reserve is developed, and afterwards padding the same in a solution of a diazotized 4-amino-di- 140 phenylamine compound in order to produce the ground dyeing.

4. A process for producing fast color reserves 145 under ground dyeings by means of ester salts of

leuco vat dyestuffs without steaming, consisting in taking a fabric impregnated with an arylide of 2:3-hydroxy-naphthoic acid, printing thereon a reserve color containing the ester salt of leuco-  
5 dibenzpyrenequinone, aluminium chloride as oxidizing agent and an acid reacting salt, thereupon drying the material, whereby the color reserve is developed, and afterwards padding the same in a solution of a diazotized 4-amino-di-  
10 phenylamine compound in order to produce the ground dyeing.

in taking a fabric impregnated with an arylide of 2:3-hydroxy-naphthoic acid, printing thereon a reserve color, containing an ester salt of a leuco vat dyestuff, aluminium chloride as oxidizing agent and an acid reacting salt, thereupon drying the material, whereby the color reserve is developed, and afterwards padding the same in a solution of diazotized 4-amino-4'-methoxy-di-phenylamine in order to produce the ground dyeing.

80

85

PHILIPPE BRANDT,  
EMIL GUBLER,  
ERNST TSCHAN.

15 5. A process for producing fast color reserves under ground dyeings by means of ester salts of leuco vat dyestuffs without steaming, consisting

90

15

20

95

25

100

30

105

35

110

40

115

45

120

50

125

55

130

60

135

65

140

70

145

75

150